

1

2,974,026

## SOLID COMPOSITE, SMOKELESS, SLOW BURNING, LOW FLAME PROPELLANT

George W. Batchelder, Glendora, Calif., assignor, by  
mesne assignments, to Aerojet-General Corporation,  
Cincinnati, Ohio, a corporation of Ohio

No Drawing. Filed Mar. 14, 1952, Ser. No. 276,703

5 Claims. (Cl. 52—5)

This invention relates to propellants or self-combustible compositions adapted for the generation of large volumes of gas useful in the performance of work, such as jet propulsion, driving turbines, pressurizing liquids, operating mechanical pistons, and the like.

The principal object of the invention is to provide a substantially smokeless, slow burning, low flame temperature propellant that is easy to manufacture and can be produced at a relatively low cost. A further object of the invention is to provide a propellant that can be safely manufactured and does not subject the user to undue hazards.

A propellant composition of the solid type ordinarily comprises a fuel ingredient having an oxidizer intimately mixed in it so that it contains the oxygen for its own combustion. The fuel may be a combustible substance such as a resin which acts as a binder for the oxidizer which is ordinarily present in a finely divided state.

Heretofore propellant formulations have been proposed for the generation of large volumes of gas to operate turbines and the like. However, in most of the proposed propellants an objection has been that the temperature at which the gases are generated is usually too high to insure long life to the mechanical parts to which the gases are applied.

It has been proposed to use ammonium nitrate as an oxidizer in the propellant to produce low flame temperature. However, up to the present time this expedient has not been used extensively due to the nature of ammonium nitrate which undergoes physical structure changes when the substance is cycled from high temperature to low temperature or vice versa. As a result, when ammonium nitrate has been incorporated into the fuel some undesirable cracking of the propellant has occurred when the propellant is subjected to wide temperatures variation. The formation of cracks in the propellant material is undesirable as it has the effect of increasing the burning area and rate beyond what is intended; and such increased burning rate may be dangerous as it may cause an explosion.

I have discovered that this cracking of the propellant containing ammonium nitrate as an oxidizer is generally due to the fact that the fuel or binder portion of the propellant is incapable of adjusting itself to expansion or contraction to which the ammonium nitrate oxidizer is subjected when the substance is cooled or heated to cause it to undergo its transition change in physical state.

One expedient that has been proposed to minimize the transition change of ammonium nitrate, has been to stabilize the ammonium nitrate before introducing it into the propellants, and this has been done by adding modifying ingredients to the ammonium nitrate. However, such modifying ingredients have the effect of creating solid particles as the gases form and have the undesirable feature that they lower the specific impulse of the propellant charge. The existence of solid particles in the gases generated by the propellant cannot be tolerated to any great extent as it would soon interfere with the

2

satisfactory operation of the mechanism in which the gases are employed.

By my present invention I have succeeded in producing a propellant that is capable of generating large volumes of substantially solid-free gases at a low flame temperature which are smokeless and slow burning, making it particularly desirable for application to equipment such as gas turbines and the like. I have further discovered that such a propellant may be compounded by using ammonium nitrate as the oxidizer, preferably in an unstabilized form, by using as a binder for the oxidizer, a particular fuel composition which provides a high degree of toughness and flexibility, thereby enabling the binder to adjust itself to the expansion or contraction of the ammonium nitrate oxidizer when this substance undergoes changes at the various transition points.

A feature of this invention resides in the fact that the fuel contains sufficient oxygen in the molecule to insure against the formation of carbon in the form of smoke in

20 the exhaust gas. The particular fuel composition which I have discovered to have this desirable property in conjunction with ammonium nitrate is the resinous condensation product of adipic acid, maleic anhydride and di-

25 ethylene glycol to which is added methyl acrylate and styrene. Ordinary resins containing ammonium nitrate will not avoid cracking when the temperatures vary widely; but the foregoing polyester resin when provided with the styrene and methyl acrylate additive and in the following indicated proportions, is an exception which can

30 result in a substantially non-cracking propellant. The proportions of the components should be held substantially within the fairly narrow limits which have been determined, as indicated below. The adipic acid should be present in an amount of at least 4 moles adipic acid to one mole of maleic anhydride. The amount of the glycol to the combined acids (adipic acid plus maleic anhydride) should range from about 0.5 to 2 moles to 1 mole of the glycol, the preferred ratio being about 1 mole of the glycol to one mole of the combined acids.

35 40 The ratio of adipic acid to maleic anhydride may vary from about 4 to 9 moles of adipic acid to 1 mole of maleic anhydride.

Suitable polyesters are those restricted to the following ingredients and range of proportions:

|                   | Moles |
|-------------------|-------|
| Diethylene glycol | 10-11 |
| Adipic acid       | 8-9   |
| Maleic anhydride  | 1-2   |

50 An example of a particularly suitable polyester resin within the foregoing range is one having the following proportions:

|    |                              |
|----|------------------------------|
| 55 | 10.5 moles diethylene glycol |
|    | 9.0 moles adipic acid        |
|    | 1.0 moles maleic anhydride   |

This resin is hereinafter referred to as Resin A.

Another somewhat similar resin found very satisfactory 60 for use in formulating the propellant is one having the following proportions:

|    |                              |
|----|------------------------------|
| 65 | 10.5 moles diethylene glycol |
|    | 8.0 moles adipic acid        |
|    | 2.0 moles maleic anhydride   |

This resin will hereinafter be referred to as Resin B.

The condensation process by which the polyester is formed is briefly as follows:

70 The ingredients comprising the adipic acid, maleic anhydride, and diethylene glycol are mixed together and heated to a temperature of approximately 140° C. until

the water formed by the reaction is substantially driven away. This is carried out in an atmosphere of inert gas such as hydrogen, nitrogen, carbon dioxide, helium, etc. When the water has been substantially removed the reaction product may then be subjected to a higher temperature not to exceed about 250° C. and preferably between 200° C. and 230° C. The condensation is continued until the polyester has reached a desired degree of polymerization which may be determined either by ascertaining the acid number in the mixture or by measuring the viscosity of the resin. The preferred degree of polymerization lies between 5 and 100 and will usually take around 70 hours of condensation. The resulting product is generally a viscous liquid which can be cooled and stored, making it available for further polymerization with the additives.

The propellant is compounded by mixing the polyester resin, the styrene and the methyl acrylate together with sufficient quantities of ammonium nitrate in finely divided form to provide enough oxygen for the complete combustion of the fuel elements. To the ammonium nitrate there is preferably added a small percentage of ammonium dichromate to improve the burning qualities of the propellant mixture. The substances are mixed together homogeneously and to the mixture there is preferably added the usual polymerization catalysts and accelerators such as methyl ethyl ketone peroxide and cobalt octoate. It is also desirable to add a small amount of lecithin to the mixture to insure a more castable homogeneous mixture.

The proportion in which the components may be admixed with each other to form satisfactory propellants are as follows:

|                              | Percent by weight |
|------------------------------|-------------------|
| Resin A or Resin B           | 4-14              |
| Styrene                      | 1-6               |
| Methyl acrylate              | 4-16              |
| Ammonium nitrate             | 65-80             |
| Ammonium dichromate          | 1-5               |
| Methyl ethyl ketone peroxide | 0.1-1.0           |
| Cobalt octoate               | 0.01-0.10         |
| Lecithin                     | 0.01-0.5          |

A specific formulation which has been found particularly satisfactory for this purpose is as follows:

|                                     | Percent by weight |
|-------------------------------------|-------------------|
| Resin A                             | 10.00             |
| Styrene                             | 2.30              |
| Methyl acrylate                     | 12.40             |
| Ammonium nitrate                    | 72.80             |
| Ammonium dichromate                 | 2.00              |
| Methyl ethyl ketone peroxide        | 0.30              |
| Cobalt octoate (1% cobalt solution) | 0.25              |
| Lecithin                            | 0.05              |
| Total                               | 100.00            |

The advantage of the above propellant formulations is that it is possible to make propellants capable of generating large volumes of substantially solid-free gases at relatively low temperatures and at the same time employ the inexpensive oxidizing component, ammonium nitrate, without the danger of having the propellant mass become cracked if subjected to a change in temperature which would normally cause the ammonium nitrate to pass through one of its many transition points and expand or contract in an amount sufficient to develop a separation within the propellant charges.

We claim:

1. A substantially smokeless, slow burning, low flame temperature propellant comprising from 4 to 14% by weight based on the weight of the total propellant of a polyester resin obtained by condensing 10 to 11 moles of diethylene glycol with from 8 to 9 moles of adipic

acid and 1 to 2 moles of maleic anhydride; from 1 to 6% by weight styrene based on the weight of the total propellant; from 4 to 16% by weight methyl acrylate based on the weight of the total propellant; from 65 to 80% by weight ammonium nitrate based on the weight of the total propellant; from 1 to 5% by weight ammonium dichromate based on the weight of the total propellant; from 0.1% to 1.0% by weight methyl ethyl ketone peroxide based on the weight of the total propellant; from 0.01 to .10% by weight cobalt octoate based on the weight of the total propellant; and from .01 to 0.5% by weight lecithin based on the weight of the total propellant.

2. A substantially smokeless, slow burning, low flame temperature propellant comprising from 4 to 14% by weight based on the weight of the total propellant of a polyester resin obtained by condensing 8 moles adipic acid, 2 moles maleic anhydride, 10½ moles diethylene glycol; from 1 to 6% by weight styrene based on the weight of the total propellant; from 4 to 16% by weight methyl acrylate based on the weight of the total propellant; from 65 to 80% by weight ammonium nitrate based on the weight of the total propellant; from 1 to 5% by weight ammonium dichromate based on the weight of the total propellant; from 0.1 to 1.0% by weight methyl ethyl ketone peroxide based on the weight of the total propellant; from 0.01 to .10% by weight cobalt octoate based on the weight of the total propellant; and from .01 to 0.5% by weight lecithin based on the weight of the total propellant.

3. A substantially smokeless, slow burning, low flame temperature propellant comprising from 4 to 14% by weight, based on the weight of the total propellant of a polyester resin obtained by condensing 10½ moles of diethylene glycol with 1 mole maleic anhydride and 9 moles adipic acid; from 1 to 6% by weight styrene based on the weight of the total propellant; from 4 to 16% by weight methyl acrylate based on the weight of the total propellant; from 65 to 80% by weight ammonium nitrate based on the weight of the total propellant; from 1 to 5% by weight ammonium dichromate based on the weight of the total propellant; from 0.1 to 1.0% by weight methyl ethyl ketone peroxide based on the weight of the total propellant; from 0.01 to .10% by weight cobalt octoate based on the weight of the total propellant; and from .01 to 0.5% by weight lecithin based on the weight of the total propellant.

4. A substantially smokeless, slow burning, low flame temperature propellant comprising 10% by weight based on the weight of the total propellant of a polyester resin obtained by condensing 8 moles of adipic acid, 2 moles of maleic anhydride and 10½ moles of diethylene glycol; 2.30% by weight styrene based on the weight of the total propellant; 12.40% by weight methyl acrylate based on the weight of the total propellant; 72.80% by weight ammonium nitrate based on the weight of the total propellant; 2% by weight ammonium dichromate based on the weight of the total propellant; 0.30% by weight methyl ethyl ketone peroxide based on the weight of the total propellant; 0.25% by weight cobalt octoate (1% cobalt solution) based on the weight of the total propellant; and 0.05% by weight lecithin based on the weight of the total propellant.

5. A substantially smokeless, slow burning, low flame temperature propellant comprising 10% by weight based on the weight of the total propellant of a polyester resin obtained by condensing 10½ moles of diethylene glycol with 1 mole maleic anhydride and 9 moles adipic acid; 2.30% by weight styrene based on the weight of the total propellant; 12.40% by weight methyl acrylate based on the weight of the total propellant; 72.80% by weight ammonium nitrate based on the weight of the total propellant; 2% by weight ammonium dichromate based on the weight of the total propellant; 0.30% by weight methyl ethyl ketone peroxide based on the weight of the total propellant.

the total propellant; 0.25% by weight cobalt octoate (1% cobalt solution) based on the weight of the total propellant; and 0.05% by weight lecithin based on the weight of the total propellant.

References Cited in the file of this patent

UNITED STATES PATENTS

2,067,234 Gordon et al. ----- Jan. 12, 1937

|           |                     |               |
|-----------|---------------------|---------------|
| 2,155,499 | Lawson -----        | Apr. 25, 1939 |
| 2,195,965 | Holm -----          | Apr. 2, 1940  |
| 2,305,224 | Patterson -----     | Dec. 15, 1942 |
| 2,319,799 | D'Alelio -----      | May 25, 1943  |
| 2,388,319 | Fuller -----        | Nov. 6, 1945  |
| 2,406,227 | King -----          | Aug. 20, 1946 |
| 2,434,872 | Taylor et al. ----- | Jan. 20, 1948 |
| 2,479,828 | Geckler -----       | Aug. 23, 1949 |